

## UNITED STATES PATENT OFFICE.

JAMES G. WEST, OF PITTSBURGH, PENNSYLVANIA.

## METHOD OF PRODUCING COKE.

No Drawing.

Application filed February 16, 1922. Serial No. 537,088.

*To all whom it may concern:*

Be it known that I, JAMES G. WEST, residing at Pittsburgh, in the county of Allegheny and State of Pennsylvania, a citizen of the United States, have invented or discovered certain new and useful Improvements in Methods of Producing Coke, of which improvements the following is a specification.

10 My invention relates to improvements in the coking of coal, and its object is the production from bituminous coal of high volatile content (a content so high that but for my invention, the material would be 15 inferior for the end in view) metallurgical coke,—coke, that is to say, serviceable in the blast furnace in the smelting of iron ore. This application is in part a continuation of an application filed by me 20 November 26, 1920, Serial No. 426,510.

There are certain ideals in the quality of coke, particularly as regards physical characteristics, which are realized in the cokes produced from coals of certain quality, 25 found in certain favored regions, and to these ideals the cokes produced from coals of less favored regions approach in different degrees of proximity. The natural supply of the best coals is of course diminishing 30 and their value is increasing.

It appears that, following methods of coking hitherto in vogue, and speaking of Pennsylvania coals at least, coals whose volatile content approaches but does not exceed 35 31% afford coke best suited for blast-furnace use; and that cokes produced from coals of higher volatile are relatively soft, do not serve so well in the blast furnace, and, besides, suffer relatively great waste in handling. My invention is directed to making 40 available as a source of good metallurgical coke, coals which because of high volatile content are otherwise unsuitable, or at least inferior, for that purpose.

45 I find, and herein lies my invention, that by taking a quantity of high volatile coal and subjecting it to distillation and continuing distillation until a portion, but a portion only, of its volatile content has been 50 driven off, while the mass under treatment still retains volatile ingredients in substantial quantity and in consequence still possesses certain physical characteristics; then cooling the mass, crushing it and mix-

ing it with new quantities of cokable material, and finally coking the mixture, carrying the operation this time through to the end.—I find that by doing so I obtain coke adequate for blast-furnace use, that is to say metallurgical coke of high quality.

The raw material may vary in volatile content. As I have said, I contemplate working with coal whose volatile content is so great that by methods hitherto in vogue only weak and inferior coke can be produced. The limit here is a fluctuating one; but, dealing with Pennsylvania coals as example, it may be given with reasonable precision as 31%. The coal with which I have achieved my invention is Pennsylvania coal 70 whole volatile content amounts to 32-34%.

The initial operation is essentially one of distillation; it should be performed in a retort oven, in order that the desired initial removal of volatile matter may be achieved 75 without any burning of the mass under treatment. The degree to which this initial step of partial removal of the volatile content, may advance admits of some latitude, and is not susceptible to precise definition in 80 figures. By way of example and still referring to the Pennsylvania coal with which I have achieved my invention, I preferably reduce the volatile content to 17-20%; I

have reason to believe that with this coal 85 the volatile content may be reduced to 10% and the invention still be enjoyed, but that it may not be reduced to 6%. But different coals will under proof show different figures. The important thing is the physical character and condition of the mass at the point where cooling interrupts the progress of distillation. It is impossible to see and discern conditions as they then are, but cooling will leave a mass, not brittle 90 and friable, like soft coke, but tough and cellular. Particles crushed between thumb and finger will give a smudge. The condition and appearance generally are such as to indicate that at the moment of suspension of distillation the mass was still melted and gummy and foaming in character.

The cooling of the charge of partially coked material, the drawing and crushing, 105 may be accomplished in usual and familiar manner. So with the mixing of the intermediate product with new quantities of

cokable material, usual methods may be pursued, grinding may precede or may follow mixing, or partial grinding before mixing may be followed by further grinding after. Ordinarily the new quantities of cokable material will be of raw coal, and ordinarily they will be of the same coal as that with which beginning was made. But of course the blending of different coal is not forbidden.

The result of mixing will be a mass which as a whole possesses a volatile ingredient approximately that of the ideal coal mentioned above—28% or thereabouts. In my work upon Pennsylvania coal it appeared that the additions of raw coal to the intermediate product exceeded the intermediate product in quantity, and this condition will I believe obtain in all practical operations.

The ultimate coking operation may be performed in a coke oven of any preferred type—retort or open-burning. I prefer, however, to complete the operation in a retort oven. This ultimate step will be the typical coking operation, practiced as upon the usual furnace charge.

If the initial step of distillation be carried beyond a certain point which, in Pennsylvania coal at least, lies somewhere from 6% to 10% volatile, the substance will begin to assume the physical characteristics of coke, that is to say when cold it will have gained greatly in hardness, and will begin to possess that metallic ring when struck with which anyone acquainted with coke is familiar.

When dealing with coal of given grade, simple and obvious tests will indicate, to what extent exactly the initial distillation may with best results be carried, and in what proportions precisely the ultimate coke oven charge should be compounded. I have indicated general conditions, compliance with which will achieve success. I add, by way of illustration, specific figures of a particular operation. The raw coal used in this illustrative operation is one having a volatile content of 34%. By the initial step of distillation the volatile content is reduced to 17%. The product of the initial distillation is mixed with more of the same raw coal in the ratio of 1:3. The regular coking operation follows. This regular coking operation I preferably perform in a retort oven, but as I have said it may be performed in an oven of any preferred type.

I am aware that proposals have heretofore been made to coke coals by two-step processes. These proposals have for the most part at least concerned the production of briquettes for use as domestic fuel, and have involved mechanical pressure upon the mass under treatment as an essential condition of operation. They have come to nothing. Certainly they have had no value nor

effect at all in the art of producing metallurgical coke,—an art which is highly specialized, and whose requirements are exacting. These earlier proposals to which I here allude have taught the art of producing metallurgical coke nothing, and could teach nothing; for, as I have learned by experimentation and study, it is necessary to succeed, so far as metallurgical coke is concerned, that in the ultimate oven charge both components of the mixture shall have volatile contents of substantial proportion; in the ultimate coking operation every ingredient particle of the mixture must under heat be changed; its fusible content must melt and integrate with the fused content of the whole. Thus and thus only does the way open to reach a practical result, so far at least as the production of metallurgical coke is concerned. The earlier proposals to which I allude have not recognized the importance and necessity of this detail of procedure. Nor have these earlier proposals involved any certain teaching as to the proportions in which the initially treated material shall be mixed with fresh quantities of raw material.

I have found the first condition essential to success to be that the initial step shall be a partial distillation; that the intermediate product shall still retain a substantial content of volatile matter; that at distillation temperature it shall still be fusible and shall become a gummy foaming mass. Incidentally I find, and I believe it to be an essential condition to success that in mixing the intermediate material with fresh quantities of raw coal, the new material shall not be less in quantity than the already treated intermediate product.

I claim as my invention:

1. The method herein described of producing from high volatile coal metallurgical coke which consists in subjecting a body of such coal to distillation, and while the material under treatment is still a fused and gummy mass, cooling it, then crushing and mixing the material with another body of cokable material, and coking the mixture to the end.

2. The method herein described of producing from high volatile coal metallurgical coke which consists in subjecting a body of such coal to distillation, and while the material under treatment is still a fused and gummy mass, cooling it, then crushing the so treated material and mixing it with another body of the same material in raw state, and coking the mixture to the end.

3. The method herein described of producing from high volatile coal metallurgical coke which consists in subjecting a body of such coal to distillation, and while the material under treatment is still a fused and gummy mass cooling it, then crushing the

so treated material and mixing it with an at least equal mass of unmodified coal, and coking the mixture.

4. The method herein described of producing from high volatile coal metallurgical coke which consists in subjecting a body of such coal to distillation and by distillation reducing its volatile content to a value not

less than 6%, then cooling the mass, and mixing with it an at least equal quantity of 10 raw coal, and finally coking the mixture.

In testimony whereof I have hereunto set my hand.

JAMES G. WEST.

Witness:

R. H. LAUTZ.